



US007267623B2

(12) **United States Patent**  
**Manami et al.**

(10) **Patent No.:** **US 7,267,623 B2**  
(45) **Date of Patent:** **Sep. 11, 2007**

(54) **GOLF BALL**

(75) Inventors: **Toshihiko Manami**, Chichibu (JP); **Eiji Takehana**, Chichibu (JP)

(73) Assignee: **Bridgestone Sports Co., Ltd.**, Tokyo (JP)

(\*) Notice: Subject to any disclaimer, the term of this patent is extended or adjusted under 35 U.S.C. 154(b) by 0 days.

(21) Appl. No.: **11/271,791**

(22) Filed: **Nov. 14, 2005**

(65) **Prior Publication Data**

US 2007/0111821 A1 May 17, 2007

(51) **Int. Cl.**

**A63B 37/12** (2006.01)

(52) **U.S. Cl.** ..... **473/378**

(58) **Field of Classification Search** ..... **473/378,**  
..... **473/351**

See application file for complete search history.

(56) **References Cited**

U.S. PATENT DOCUMENTS

5,029,870 A \* 7/1991 Concepcion et al. ..... 473/378

5,506,292 A \* 4/1996 Horiuchi et al. ..... 524/430  
6,194,505 B1 2/2001 Sone et al.  
6,642,314 B2 11/2003 Sone et al.  
2004/0147694 A1 7/2004 Sone et al.

FOREIGN PATENT DOCUMENTS

|    |               |         |
|----|---------------|---------|
| JP | 11-35633 A    | 2/1999  |
| JP | 11-164912 A   | 6/1999  |
| JP | 3293679 B2    | 4/2002  |
| JP | 3293694 B2    | 4/2002  |
| JP | 2002-293996 A | 10/2002 |
| JP | 3649568 B2    | 2/2005  |

\* cited by examiner

Primary Examiner—Raeann Trimiew

(74) Attorney, Agent, or Firm—Sughrue Mion, PLLC

(57) **ABSTRACT**

In a golf ball composed of a core and a cover of one or more layer that encloses the core, at least one layer of the cover is composed of 100 parts by weight of a base resin, 1 to 7 parts by weight of titanium oxide, 0.002 to 0.4 part by weight of a blue pigment, and 0.0006 to 0.5 part by weight of a violet pigment. The weight ratio of the blue pigment to the violet pigment is from 1:99 to 99:1. A sufficient whiteness is imparted to the surface of the ball, and the ball has an excellent resistance to color fading.

**11 Claims, No Drawings**

**1**  
**GOLF BALL**

BACKGROUND OF THE INVENTION

The present invention relates to golf balls, such as two-piece solid golf balls and three-piece solid golf balls, which are composed of a core and a cover of one or more layer that encloses the core.

Many innovations, such as including within the core and cover portions of the golf ball, or in a clear coating, various color pigments (e.g., blue pigments, violet pigments, red pigments) have hitherto been disclosed for preventing to the extent possible the decline in whiteness that occurs at the surface of a golf ball which is repeatedly used and thereby maintaining a good ball appearance. Such golf balls are described in, for example, JP Pat. No. 3,649,568, JP Pat. No. 3,293,679, JP Pat. No. 3,293,694 and JP-B 4-50029.

JP Pat. No. 3,649,568, which relates to a golf ball, describes a means for conferring a high degree of whiteness without using white paint that involves incorporating specific amounts of a blue pigment and a red pigment into a cover made of an ionomer resin. However, when such a golf ball is used over an extended period of time, the color at the surface of the ball fades due to exposure to direct sunlight and other reasons. Hence, further improvements in such properties as resistance to color fading have been desired.

JP Pat. No. 3,293,679 and JP Pat. No. 3,293,694 disclose the use, as the core material in a golf ball, of a white rubber composition obtained by compounding specific amounts of titanium oxide, blue pigment and violet pigment in a golf ball core-forming rubber composition. However, the resulting one-piece golf ball, while useful on a practice range, is unfit for competitive use.

JP-B 4-50029 discloses, in a golf ball having a cover made of balata rubber, the addition of small amounts of a component which exhibits a blue color and a component which exhibits a violet color to the base resin of a white coating so as to impart a white appearance to the balata cover. However, when the cover is painted white to achieve sufficient whiteness, scuffing of the ball causes the underlying material to become visible, compromising the appearance of the ball.

SUMMARY OF THE INVENTION

It is thus an object of the invention to provide a golf ball in which sufficient whiteness is conferred to the surface of the ball and which has an improved resistance to color fading.

As a result of extensive investigations, we have discovered that, in a golf ball composed of a core and a cover of one or more layer that encloses the core, by having at least one layer of the cover composed of 100 parts by weight of a base resin, 1 to 7 parts by weight of titanium oxide, 0.002 to 0.4 part by weight of a blue pigment and 0.0006 to 0.5 part by weight of a violet pigment, and by setting the weight ratio of the blue pigment to the violet pigment to from 1:99 to 99:1, the degree of whiteness of the cover itself is enhanced so that, even with use over an extended period of time, the surface of the ball can be kept sufficiently white, in addition to which the color fading resistance can be improved.

That is, we have found that by employing a violet pigment instead of the red pigment used in the prior-art cover materials formulated with specific amounts of titanium white, blue pigment and red pigment, mixture with the base

**2**

resin gives the ball an unexpectedly vivid whiteness, in addition to which the color of the ball does not fade with prolonged use of the ball.

Accordingly, the invention provides the following golf balls.

- [1] A golf ball composed of a core and a cover of one or more layer that encloses the core, the ball being characterized in that at least one layer of the cover is composed of 100 parts by weight of a base resin, 1 to 7 parts by weight of titanium oxide, 0.002 to 0.4 part by weight of a blue pigment and 0.0006 to 0.5 part by weight of a violet pigment, wherein the weight ratio of the blue pigment to the violet pigment is from 1:99 to 99:1.
- [2] The golf ball of [1] above, wherein the base resin of the cover is composed primarily of a thermoplastic resin and/or a thermoplastic elastomer.
- [3] The golf ball of [2] above, wherein the thermoplastic resin is an ionomer resin.
- [4] The golf ball of [1] above, wherein the at least one layer of the cover additionally contains from 0.0001 to 0.01 part by weight of a yellow pigment per 100 parts by weight of the base resin.
- [5] The golf ball of [1] above, wherein the cover is coated on a surface thereof with a clear urethane coating.
- [6] The golf ball of [1] above, wherein the weight ratio of the blue pigment to the violet pigment is from 5:95 to 95:1.
- [7] The golf ball of [1] above, wherein the weight ratio of the blue pigment to the violet pigment is from 10:90 to 90:10.

DETAILED DESCRIPTION OF THE INVENTION

The invention is described more fully below.

The invention is a golf ball composed of a core and a cover of one or more layer that encloses the core, wherein at least one layer of the cover is composed of specific amounts of a base resin, titanium oxide, a blue pigment and a violet pigment.

The core can be made from a rubber composition which includes such ingredients as a co-crosslinking agent, an organic peroxide, an inert filler and an organosulfur compound. The base rubber in the rubber composition is preferably a polybutadiene.

It is advantageous for the polybutadiene used as the rubber component to have on the polymer chain thereof a cis-1,4 bond content of at least 60 wt %, preferably at least 80 wt %, more preferably at least 90 wt %, and most preferably at least 95 wt %. If cis-1,4 bonds account for too low a proportion of the bonds on the polybutadiene molecule, the rebound of the golf ball may decrease.

The polybutadiene has a 1,2-vinyl bond content, based on the polymer chain, of generally 2% or less, preferably 1.7% or less, and more preferably 1.5% or less. If the 1,2-vinyl bond content is too high, the resilience may decrease.

To obtain a vulcanized molding of the rubber composition having a good resilience, the above-described polybutadiene used in the invention is preferably synthesized with a rare-earth catalyst or a group VIII metal compound catalyst, and most preferably synthesized with a rare-earth catalyst.

The rare-earth catalyst is not subject to any particular limitation. Illustrative examples include catalysts made up of a combination of a lanthanide series rare-earth compound, an organoaluminum compound, an alumoxane, a halogen-bearing compound and an optional Lewis base.

Examples of suitable lanthanide series rare-earth compounds include halides, carboxylates, alcohohlates, thioalcohohlates and amides of atomic number 57 to 71 metals.

In the practice of the invention, the use of a neodymium catalyst in which a neodymium compound serves as the lanthanide series rare-earth compound is particularly advantageous because it enables a polybutadiene rubber having a high cis-1,4 content and a low 1,2-vinyl content to be obtained at an excellent polymerization activity. Suitable examples of such rare-earth catalysts include those mentioned in JP-A 11-35633, JP-A 11-164912 and JP-A 2002-293996.

To enhance the resilience, it is preferable for the polybutadiene synthesized using the lanthanide series rare-earth compound catalyst to account for at least 10 wt %, preferably at least 20 wt %, and most preferably at least 40 wt %, of the rubber components.

Rubber components other than the above-described polybutadiene may be included in the base rubber insofar as the objects of the invention are attainable. Illustrative examples of rubber components other than the above-described polybutadiene include other polybutadienes, and other diene rubbers such as styrene-butadiene rubber, natural rubber, isoprene rubber and ethylene-propylene-diene rubber.

Examples of co-crosslinking agents include unsaturated carboxylic acids and the metal salts of unsaturated carboxylic acids.

Specific examples of unsaturated carboxylic acids include acrylic acid, methacrylic acid, maleic acid and fumaric acid. Acrylic acid and methacrylic acid are especially preferred.

The metal salts of unsaturated carboxylic acids, while not subject to any particular limitation, are exemplified by the above-mentioned unsaturated carboxylic acids neutralized with a desired metal ion. Specific examples include the zinc and magnesium salts of methacrylic acid and acrylic acid. The use of zinc acrylate is especially preferred.

The unsaturated carboxylic acid and/or metal salt thereof is included in an amount, per 100 parts by weight of the base rubber, of at least 10 parts by weight, preferably at least 15 parts by weight, and more preferably at least 20 parts by weight, but not more than 60 parts by weight, preferably not more than 50 parts by weight, more preferably not more than 45 parts by weight, and most preferably not more than 40 parts by weight. Too much may make the core too hard, giving the ball an unpleasant feel on impact, whereas too little may lower the rebound of the ball.

The organic peroxide may be a commercially available product, suitable examples of which include Percumil D (produced by NOF Corporation), Perhexa 3M (NOF Corporation), and Luperco 231XL (Atochem Co.). These may be used singly or as a combination of two or more thereof.

The amount of organic peroxide included per 100 parts by weight of the base rubber is at least 0.1 part by weight, preferably at least 0.3 part by weight, more preferably at least 0.5 part by weight, and most preferably at least 0.7 part by weight, but not more than 5 parts by weight, preferably not more than 4 parts by weight, more preferably not more than 3 parts by weight, and most preferably not more than 2 parts by weight. Too much or too little organic peroxide may make it impossible to achieve a ball having suitable feel on impact, durability and rebound.

Examples of suitable inert fillers include zinc oxide, barium sulfate and calcium carbonate. These may be used singly or as a combination of two or more thereof.

The amount of inert filler included per 100 parts by weight of the base rubber is at least 1 part by weight, and preferably at least 5 parts by weight, but not more than 50 parts by weight, preferably not more than 40 parts by weight, more preferably not more than 30 parts by weight, and most

preferably not more than 20 parts by weight. Too much or too little inert filler may make it impossible to achieve a proper weight and a suitable rebound.

In addition, an antioxidant may be included if necessary. Illustrative examples of suitable commercial antioxidants include Nocrac NS-6, Nocrac NS-30 (both available from Ouchi Shinko Chemical Industry Co., Ltd.), and Yoshinox 425 (available from Yoshitomi Pharmaceutical Industries, Ltd.). These may be used singly or as a combination of two or more thereof.

The amount of antioxidant included per 100 parts by weight of the base rubber is 0 or more part by weight, preferably at least 0.05 part by weight, more preferably at least 0.1 part by weight, and most preferably at least 0.2 part by weight, but not more than 3 parts by weight, preferably not more than 2 parts by weight, more preferably not more than 1 part by weight, and most preferably not more than 0.5 part by weight. Too much or too little antioxidant may make it impossible to achieve a suitable rebound and durability.

To enhance the rebound of the golf ball and increase its initial velocity, it is preferable to include within the core an organosulfur compound.

No particular limitation is imposed on the organosulfur compound, provided it improves the rebound of the golf ball. Exemplary organosulfur compounds include thiophenols, thionaphthols, halogenated thiophenols, and metal salts thereof. Specific examples include pentachlorothiophenol, pentafluorothiophenol, pentabromothiophenol, p-chlorothiophenol, the zinc salt of pentachlorothiophenol, the zinc salt of pentafluorothiophenol, the zinc salt of pentabromothiophenol, the zinc salt of p-chlorothiophenol; and diphenylpolysulfides, dibenzylpolysulfides, dibenzoylpolysulfides, dibenzothiazoylpolysulfides and dithiobenzoylpolysulfides having 2 to 4 sulfurs. Diphenyldisulfide and the zinc salt of pentachlorothiophenol are especially preferred.

To enhance the rebound of the golf ball and increase its initial velocity, it is preferable to include within the core an organosulfur compound.

It is recommended that the amount of the organosulfur compound included per 100 parts by weight of the base rubber be at least 0.05 part by weight, and preferably at least 0.1 part by weight, but not more than 5 parts by weight, preferably not more than 4 parts by weight, more preferably not more than 3 parts by weight, and most preferably not more than 2.5 parts by weight. If too much organosulfur compound is included, the effects of addition may peak so that further addition has no apparent effect, whereas the use of too little organosulfur compound may fail to confer the effects of such addition to a sufficient degree.

It is preferable for the core to have a diameter of at least 32.0 mm, and especially at least 33.0 mm, but not more than 40.5 mm, and especially not more than 39.5 mm. In addition, it is preferable for the core to have a weight of 23 to 40 g, and especially 25 to 38 g.

Here, the core, within the above diameter range, has a compressive deflection when subjected to loading from an initial load of 10 kgf to a final load of 130 kgf (hardness under loading from 10 to 130 kgf) of at least 2 mm, and preferably at least 3 mm, but not more than 6 mm, and preferably not more than 5 mm. If the amount of deformation is too small, the ball will have a hard feel on impact. In addition, the spin rate will increase, which may shorten the carry of the ball when hit at a low head speed with a driver (W#1) or when struck with an iron. On the other hand, if the amount of deformation is too large, the durability of the ball

to cracking on repeated impact may worsen and the rebound may decrease, resulting in a shorter than desirable carry.

The type of core used in the invention is not subject to any particular limitation. Examples of various cores that may be used include solid cores for two-piece balls, solid cores having a plurality of vulcanized rubber layers, solid cores having a plurality of resin layers, and thread-wound cores having a rubber thread layer.

The core may be formed by a method in which a rubber composition composed primarily of the above-described base rubber is vulcanized and cured by a known method to give a spherical vulcanized and molded core. Vulcanization may be carried out at a temperature of 100 to 200° C. and over a period of 10 to 40 minutes.

Next, the cover of one or more layer which encloses the core is described.

The base resin of the cover in the invention is composed primarily of at least one selected from among thermoplastic resins and thermoplastic elastomers. At least one selected from among thermoplastic block copolymers, polyester elastomers, polyamide elastomers, polyurethane elastomers and ionomer resins may be suitably used. The use of an ionomer resin is especially preferred.

Suitable thermoplastic block copolymers include those in which the hard segments are made of crystalline polyethylene blocks (C) and/or crystalline polystyrene blocks (S); and the soft segments are made of polybutadiene blocks (B), polyisoprene blocks (I), blocks of a relatively random copolymer of ethylene and butylene (EB) or blocks of a relatively random copolymer of ethylene and propylene (EP), preferably blocks of a relatively random copolymer of ethylene and butylene (EB) or blocks of a relatively random copolymer of ethylene and propylene (EP), and most preferably blocks of a relatively random copolymer of ethylene and butylene (EB).

Illustrative examples of such thermoplastic block copolymers include S-EB-S, S-B-S, S-I-S, S-EB, S-EB-S-EB, S-EP-S, S-EB-C, S-B-C, S-I-C, S-EP-C, C-EB-C, C-B-C, C-I-C, C-EB, C-EB-C-EB, and C-EP-C. Selecting crystalline polystyrene blocks (S) as the hard segments is advantageous from the standpoint of moldability, and including crystalline polyethylene blocks (C) as the hard segments is advantageous from the standpoint of rebound.

If the thermoplastic block copolymer is a C-EB-C or S-EB-C type block copolymer, it can be obtained by hydrogenating butadiene or a styrene-butadiene copolymer.

A polybutadiene in which bonding within the butadiene structure is characterized by the presence of block-like 1,4-polymer regions having a 1,4-bond content of at least 95 wt %, and in which the butadiene structure as a whole has a 1,4-bond content of at least 50 wt %, and preferably at least 80 wt %, may be suitably used here as the polybutadiene or styrene-butadiene copolymer in hydrogenation.

The degree of hydrogenation (conversion of double bonds in the polybutadiene or styrene-butadiene copolymer to saturated bonds) in the hydrogenate is preferably 60 to 100%, and more preferably 90 to 100%. Too low a degree of hydrogenation may give rise to undesirable effects such as gelation in the blending step with other components such as an ionomer resin and, when the golf ball is formed, may compromise the weather resistance and durability to impact of the cover.

In the thermoplastic block copolymer, the content of the hard segments is preferably from 10 to 50 wt %, and more preferably from 15 to 50 wt %. If the content of hard segments is too high, the cover may lack sufficient flexibility, making it difficult to effectively achieve the objects of

the invention. On the other hand, if the content of hard segments is too low, the blend may have a poor moldability.

The thermoplastic block copolymer has a number-average molecular weight of preferably from 30,000 to 800,000.

5 The polyester elastomer is constructed primarily of hard segments made of a high-melting crystalline polymer composed of crystalline aromatic polyester units, and soft segments made of low-melting polymer segments composed of aliphatic polyether units and/or aliphatic polyester units.

10 Preferred examples of the high-melting crystalline polymer include polybutylene terephthalates derived from terephthalic acid and/or dimethyl terephthalate in combination with 1,4-butanediol. Other illustrative examples include polyesters derived from a dicarboxylic acid component such as isophthalic acid, phthalic acid, naphthalene-2,6-dicarboxylic acid, naphthalene-2,7-dicarboxylic acid, diphenyl-4,4'-dicarboxylic acid, diphenoxycarboxylic acid, 5-sulfoisophthalic acid, or ester-forming derivatives thereof in combination with a diol having a molecular weight of up to 300, such as an aliphatic diol (e.g., ethylene glycol, trimethylene glycol, pentamethylene glycol, hexamethylene glycol, neopentyl glycol, decamethylene glycol), alicyclic diol (e.g., 1,4-cyclohexanedimethanol, tricyclodecanedimethanol), or aromatic diol (e.g., xylylene glycol, bis(p-hydroxy)phenyl, bis(p-hydroxyphenyl)propane, 2,2-bis[4-(2-hydroxyethoxy)phenyl]propane, bis[4-(2-hydroxyethoxy)phenyl]sulfone, 1,1-bis[4-(2-hydroxyethoxy)phenyl]cyclohexane, 4,4'-dihydroxy-p-terphenyl, and 4,4'-dihydroxy-p-phenylphenyl). Use can also be made of 15 copolymeric polyesters prepared from two or more of these dicarboxylic acid components and diol components. In addition, polycarboxylic acid components, polyoxy acid components and polyhydroxy components having a functionality of three or more can be copolymerized therein 20 to 35 within a range of up to 5 mol %.

As noted above, the low-melting polymer segments are composed of aliphatic polyether units and/or aliphatic polyester units.

Illustrative examples of the aliphatic polyether include 40 poly(ethylene oxide) glycol, poly(propylene oxide) glycol, poly(tetramethylene oxide) glycol, poly(hexamethylene oxide) glycol, copolymers of ethylene oxide and propylene oxide, ethylene oxide addition polymers of poly(propylene oxide) glycols, and copolymers of ethylene oxide and tetrahydrofuran.

Illustrative examples of the aliphatic polyester include poly( $\epsilon$ -caprolactone), polyantholactone, polycaprylolactone, poly(butylene adipate) and poly(ethylene adipate).

The thermoplastic block copolymer has a melt index at 50 230° C. of preferably 0.5 to 15 g/10 min, and more preferably 1 to 7 g/10 min. Outside of this range, problems such as weld lines, sink marks and short shots may arise during injection molding.

In terms of the elastic properties of the resulting polyester 55 block copolymer, poly(tetramethylene oxide) glycol, ethylene oxide addition polymers of poly(propylene oxide) glycol, poly( $\epsilon$ -caprolactone), poly(butylene adipate) and poly(ethylene adipate) are preferred. Poly(tetramethylene oxide) glycol is especially preferred.

60 The low-melting polymer segments have a number-average molecular weight in the copolymerized state of preferably about 300 to 6,000.

Letting the combined amount of high-melting crystalline 65 polymer segments and low-melting polymer segments which are copolymerized to form the polyester elastomer be 100 wt %, it is advantageous for the polyester elastomer to include at least 15 wt %, and preferably at least 50 wt %, but

not more than 90 wt %, of the low-melting polymer segments. At a proportion of low-melting polymer segments higher than the above range, adequate melt characteristics suitable for injection molding may not be attainable, which can make it difficult to achieve uniform mixture during melt blending with the other components. On the other hand, if the proportion is too low, sufficient flexibility and rebound may not be achieved.

The above-described polyester elastomer is a copolymer composed primarily of the foregoing high-melting crystalline polymer segments and low-melting polymer segments. Any suitable known method may be used without particular limitation to prepare the polyester elastomer. Examples of preferred methods of preparation include methods (i) to (v) below.

- (i) A method in which a lower alcohol diester of a dicarboxylic acid, an excess amount of low-molecular-weight glycol, and the low-melting polymer segment components are subjected to transesterification in the presence of a catalyst, and the resulting reaction products are polycondensed.
- (ii) A method in which a dicarboxylic acid, an excess amount of a glycol and the low-melting polymer segment components are subjected to esterification in the presence of a catalyst, and the resulting reaction products are polycondensed.
- (iii) A method in which first the high-melting crystalline segments are prepared, then the low-melting segment components are added thereto and subjected to a transesterification reaction to effect randomization.
- (iv) A method in which the high-melting crystalline segments and the low-melting polymer segments are joined together using a chain linking agent.
- (v) In cases where poly( $\epsilon$ -caprolactone) is used as the low-melting polymer segments, a method in which the high-melting crystalline segments are subjected to an addition reaction with  $\epsilon$ -caprolactone monomer.

It is recommended that the polyester elastomer of the invention have a hardness, as measured in accordance with ASTM D-2240 (Shore D hardness), of at least 10, and preferably at least 20, but not more than 50, and preferably not more than 40.

Moreover, it is advantageous for the rebound resilience, as measured in accordance with British Standard 903 (BS 903), to be a high value of generally at least 40%, and preferably at least 50%, but not more than 90%. If the material has too low a rebound resilience, moldings of the resin composition described herein will have a low rebound, which may diminish the flight performance of golf balls made therewith.

It is desirable for the flexural rigidity, as measured in accordance with JIS K-7106, to be relatively low, with a value of at least 5 MPa, preferably at least 10 MPa, and more preferably at least 15 MPa, but not more than 250 MPa, preferably not more than 200 MPa, and even more preferably not more than 150 MPa. If the flexural rigidity is too high, the resin composition moldings of the invention will be too rigid, which may worsen the feel on impact and the durability of golf balls made therewith.

The polyamide elastomer is a thermoplastic elastomer which has on the molecule both hard segments composed of polyamide and soft segments composed of polyether.

Specific examples of thermoplastic polyamide elastomers include the product commercially available from Daicel Fuels under the trade name Daiamid PAE.

The thermoplastic polyurethane material has a morphology which includes soft segments composed of a polymeric

polyol (polymeric glycol) and hard segments composed of a chain extender and a diisocyanate. The polymeric polyol used as a starting material may be any that is employed in the art relating to thermoplastic polyurethane materials, without particular limitation. Exemplary polymeric polyols include polyester polyols and polyether polyols, although polyether polyols are better than polyester polyols for synthesizing thermoplastic polyurethane materials that provide a high rebound resilience and have excellent low-temperature properties. Suitable polyether polyols include polytetramethylene glycol and polypropylene glycol. Polytetramethylene glycol is especially preferred for achieving a good rebound resilience and good low-temperature properties. The polymeric polyol has an average molecular weight of preferably 1,000 to 5,000. To synthesize a thermoplastic polyurethane material having a high rebound resilience, an average molecular weight of 2,000 to 4,000 is especially preferred.

Preferred chain extenders include those used in the prior art relating to thermoplastic polyurethane materials. Illustrative, non-limiting examples include 1,4-butyleneglycol, 1,2-ethylene glycol, 1,3-butanediol, 1,6-hexanediol, and 2,2-dimethyl-1,3-propanediol. These chain extenders have an average molecular weight of preferably 20 to 15,000.

Diisocyanates suitable for use include those employed in the prior art relating to thermoplastic polyurethane materials. Illustrative, non-limiting, examples include aromatic diisocyanates such as 4,4'-diphenylmethane diisocyanate, 2,4-toluene diisocyanate and 2,6-toluene diisocyanate; and aliphatic diisocyanates such as hexamethylene diisocyanate. Depending on the type of isocyanate used, the crosslinking reaction during injection molding may be difficult to control. In the present invention, to ensure stability, it is most preferable to use an aromatic diisocyanate, and specifically 4,4'-diphenylmethane diisocyanate.

The most preferred thermoplastic polyurethane material is a thermoplastic polyurethane material synthesized using a polyether polyol and an aromatic diisocyanate, wherein the polyether polyol is polytetramethylene glycol having an average molecular weight of at least 2,000 and the aromatic diisocyanate is 4,4'-diphenylmethane diisocyanate.

A commercial product may be suitably used as the above-described thermoplastic polyurethane material. Illustrative examples include Pandex T-8290, Pandex T-8295 and Pandex T-8260 (all manufactured by DIC Bayer Polymer, Ltd.), and Resamine 2593 and Resamine 2597 (both manufactured by Dainichi Seika Colour & Chemicals Mfg. Co., Ltd.).

The ionomer resin may be any that has hitherto been used as a cover material in golf balls, although it is preferable to use an ionomer resin containing (1) a metal ion neutralization product of an olefin-unsaturated carboxylic acid random copolymer and/or an olefin-unsaturated carboxylic acid random copolymer, and (2) a metal ion neutralization product of an olefin-unsaturated carboxylic acid-unsaturated carboxylic acid ester random terpolymer and/or an olefin-unsaturated carboxylic acid-unsaturated carboxylic acid ester random terpolymer.

The olefins in component (1) and component (2) are preferably  $\alpha$ -olefins. Specific examples of  $\alpha$ -olefins include ethylene, propylene and 1-butene. Of these, ethylene is especially preferred. A plurality of such olefins may be used in combination.

The unsaturated carboxylic acids in component (1) and component (2) are preferably  $\alpha,\beta$ -unsaturated carboxylic acids having 3 to 8 carbon atoms. Specific examples of  $\alpha,\beta$ -unsaturated carboxylic acids having 3 to 8 carbons include acrylic acid, methacrylic acid, ethacrylic acid, ita-

conic acid, maleic acid and fumaric acid. Of these, acrylic and methacrylic acid are preferred. A plurality of these unsaturated carboxylic acids may be used in combination.

The unsaturated carboxylic acid ester in component (2) is preferably a lower alkyl ester of the foregoing unsaturated carboxylic acid. Examples include those obtained by reacting the above unsaturated carboxylic acids with a lower alcohol such as methanol, ethanol, propanol, n-butanol or isobutanol. Acrylic acid esters and methacrylic acid esters are especially preferred.

More specific examples of the unsaturated carboxylic acid ester in component (2) include methyl methacrylate, ethyl methacrylate, propyl methacrylate, butyl methacrylate, methyl acrylate, ethyl acrylate, propyl acrylate and butyl acrylate. The use of butyl acrylate (n-butyl acrylate, i-butyl acrylate) is especially preferred. A plurality of these unsaturated carboxylic acid esters may be used in combination.

When preparing the above-described olefin-unsaturated carboxylic acid copolymer and olefin-unsaturated carboxylic acid-unsaturated carboxylic acid ester copolymer, optional monomers may also be copolymerized insofar as the objects of the invention are attainable.

The content of unsaturated carboxylic acid within these copolymers is preferably from 5 to 20 wt % in above component (1), and from 1 to 10 wt % in above component (2). Too low a content of unsaturated carboxylic acid may diminish the rigidity and rebound, decreasing the flight performance of the golf ball. On the other hand, too high a content of unsaturated carboxylic acid may result in a poor flexibility.

The content of unsaturated carboxylic acid ester in component (2) is preferably from 12 to 45 wt %. If the content of unsaturated carboxylic acid ester is too low, a softening effect may not be achieved. On the other hand, if the unsaturated carboxylic acid ester content is too high, the rebound may decrease.

When above component (1) and above component (2) are blended and used together, it is advantageous for these components to be used in a weight ratio (1)/(2) of preferably 100/0 to 25/75, and more preferably 100/0 to 50/50. The use of too much component (2) may result in a less than satisfactory rebound.

The ionomer resin is preferably one obtained by neutralizing the above-described copolymer with at least one type of metal ion having a valence of 1 to 3. Examples of metal ions having a valence of 1 to 3 that are suitable for neutralization include sodium, potassium, lithium, magnesium, calcium, zinc, aluminum, ferrous ions and ferric ions.

Such metal ions may be introduced by reacting the above-described copolymers with, for example, a hydroxide, methoxide, ethoxide, carbonate, nitrate, formate, acetate or oxide of the aforementioned valence 1 to 3 metal.

It is advantageous for the carboxylic acid included within the above copolymer to be neutralized with metal ions such that at least 10 mol %, preferably at least 30 mol %, and up to 100 mol %, preferably up to 90 mol %, of the carboxyl groups on the copolymer are neutralized. A low degree of neutralization may result in a low rebound.

From the standpoint of enhancing the rebound, it is desirable to use a univalent metal ionomer and a divalent metal ionomer in admixture. The former and the latter are preferably mixed and used together at this time in a weight ratio of 20/80 to 80/20.

Also, it is known that a good balance between resilience and durability can be achieved in a layer composed primarily of ionomer resin by blending suitable amounts of

ionomer resins containing different monovalent, divalent or trivalent metal ionic species. Such blending is preferred in the practice of the invention.

The ionomer resin used in the invention may be a commercial product. Exemplary ionomer resins include Surlyn, which is produced by E.I. du Pont de Nemours and Co., Inc., and Himilan, which is produced by DuPont-Mitsui Polymers Co., Ltd.

At least one layer of the cover in the inventive golf ball 10 is composed primarily of the above-described base resin. That is, the above base resin accounts for at least 50 wt %, preferably at least 60 wt %, and more preferably at least 70 wt %, of the cover resin material.

Next, titanium oxide, a blue pigment and a violet pigment 15 are compounded with the above-described cover base resin.

The titanium oxide is titanium white. Either a rutile-type or anatase-type titanium white may be used. These may be manufactured by a suitable process such as the sulfate process or the chloride process, and may be surface treated 20 with hydrous oxides of aluminum and silicon. Use can also be made of, for example, ultrafine titanium oxide particles (particle diameter, 0.02 to 0.05  $\mu\text{m}$ ), high-purity titanium oxide, or titanium oxide needles (fiber diameter, 0.05 to 0.15  $\mu\text{m}$ ; fiber length, 3 to 12  $\mu\text{m}$ ).

25 The amount of titanium oxide used in the invention is 1 to 7 parts by weight, and preferably 2 to 5 parts by weight, per 100 parts by weight of the base resin. At less than 1 part by weight, the whiteness of the titanium oxide decreases, whereas at more than 7 parts by weight, the white color takes 30 on a yellow cast.

The blue pigment used in the invention is exemplified by inorganic blue pigments such as ultramarine blue, cobalt blue and Prussian blue; and organic blue pigments such as phthalocyanine blue, alkali blue and indanthrone blue. The 35 use of ultramarine blue is especially preferred.

The amount of the above blue pigment used is from 0.002 to 0.4 part by weight, and preferably from 0.005 to 0.05 part by weight, per 100 parts by weight of the base resin. If the 40 amount of blue pigment used is less than 0.002 part by weight, the white color becomes yellowish. On the other hand, at more than 0.4 part by weight, the white color takes on a blue tinge.

The violet pigment used in the invention is exemplified by ultramarine violet, cobalt violet, manganese violet, dioxane violet and quinacridone violet. The use of ultramarine violet 45 is especially preferred.

The amount of the above violet pigment used is from 0.0006 to 0.5 part by weight, and preferably from 0.001 to 0.1 part by weight, per 100 parts by weight of the base resin. If the amount of violet pigment is less than 0.0006 part by weight, the white color becomes yellowish, whereas at more than 0.5 wt %, the white color becomes reddish.

In addition, a yellow pigment can be added together with the above-described blue and violet pigments. Suitable examples of this yellow pigment include monoazo, diaryl, complex metal oxide and condensed azo yellow pigments. The use of titanium yellow, which is a type of complex metal oxide, is especially preferred.

Using the above yellow pigment together with the violet pigment can enhance the degree of whiteness. The amount of yellow pigment effective for this purpose is from 0.0001 to 0.01 part by weight.

The respective above-described pigments can be used in a form that has been surface treated to enhance dispersibility in the base resin, or may be used together with any of various dispersants.

## 11

The relative proportions of the above-described blue pigment and violet pigment, expressed as the weight ratio of blue pigment to violet pigment, is from 1:99 to 99:1, preferably from 5:95 to 95:5, and more preferably from 10:90 to 90:10.

If necessary, other ingredients such as dyes, pigments (e.g., titanium dioxide, zinc oxide, barium sulfate), UV absorbers, antioxidants and dispersion aids may also be included in the cover material. Dispersion aids are exemplified by polyethylene waxes, metal soaps, fatty acid esters and fatty acid amides, and may be included in an amount, based on the overall cover material composition, of at least 0.2 wt %, and preferably at least 0.5 wt %, but not more than 10.0 wt %, and preferably not more than 5 wt %.

In the practice of the invention, if the cover has two or more layers, it is suitable for the cover layer having various pigments compounded therein which is a distinctive feature of the invention to be used as the outermost layer, although use is not limited to this position. If the golf ball of the invention is a three-piece golf ball having two cover layers, the material making up the cover inner layer adjoining the outermost layer may be composed of one or more of the above-described thermoplastic resins and thermoplastic elastomers, and may be the same as or different from the material making the cover outer layer.

Formation of the cover may be carried out by a conventional method, such as a known injection molding method. For example, the golf ball may be obtained by placing the core within a given injection-molding mold, then injection molding the cover material around the core. If the cover has two or more layers, including an intermediate layer or outermost layer, a cover of two or more layers can be formed over the core by carrying out injection molding two or more times by a method similar to that described above. Alternatively, the cover may be formed by enclosing the core or an intermediate layer with two half-cups that have been molded beforehand as hemispherical shells, then molding under applied heat and pressure.

The surface of the cover on the inventive golf ball may have numerous dimples, and also markings such as a brand name and a ball number, placed thereon. Once the application of markings has been completed, the golf ball can be administered a clear coating (coated with a transparent coating) so as to protect the surface of the ball, including the positions of the markings, and to improve the appearance of the ball. Coating may be carried out using a known method, such as spraying the ball while it is perched on the tips of needles on a needle bed, to apply any of various coatings to the entire ball.

Coatings used for clear coats, while not subject to any particular limitation, can be prepared as urethane coatings having a base composed of a single resin or a mixture of two or more resins selected from among polyester, acrylic and polyether resins. To improve the wear resistance of the ball, it is desirable to use a coating in which the resin component has a molecular weight of 20,000 to 25,000 and a hydroxyl number of 100 to 200.

The golf ball of the invention (if the ball has been clear coated, "golf ball" signifies here to the surface of the ball after coating) is preferably formed to a diameter and weight in accordance with the Rules of Golf, and is generally

## 12

formed to a diameter of not less than 42.67 mm and a weight of not more than 45.93 g. The diameter is preferably from 42.67 to 42.9 mm. Deflection by the ball when subjected to a load of 980 N (100 kg) is preferably 2.0 to 4.0 mm, more preferably 2.2 to 3.8 mm, and most preferably 2.5 to 3.5 mm.

As described above, in the golf ball of the invention, a sufficient whiteness is imparted to the surface of the ball and the ball has an excellent resistance to color fading.

## EXAMPLES

The following Examples of the invention and Comparative Examples are provided by way of illustration and not by way of limitation.

## Example 1, Comparative Examples 1 and 2

In each respective example, a core material of the composition indicated in Table 1 below was masticated, then vulcanized and molded at 155° C. for 15 minutes to give a 35.3 mm diameter solid core.

TABLE 1

| Core formulation                   | Amount<br>(parts by weight) |
|------------------------------------|-----------------------------|
| BR01                               | 50                          |
| BR51                               | 50                          |
| Zinc acrylate                      | 24.0                        |
| Peroxide (1)                       | 0.6                         |
| Peroxide (2)                       | 0.6                         |
| Antioxidant                        | 0.1                         |
| Zinc salt of pentachlorothiophenol | 0.1                         |
| Zinc oxide                         | 5                           |
| Barium sulfate                     | 20.8                        |

The core materials in Table 1 are described below.

BR01: A butadiene rubber produced by JSR Corporation under the trade name BR01.

BR51: A butadiene rubber produced by JSR Corporation under the trade name BR51.

Peroxide (1): Dicumyl peroxide, produced by NOF Corporation under the trade name Percumil D.

Peroxide (2): 1,1-Bis(t-butylperoxy)-3,3,5-trimethylcyclohexane, produced by NOF Corporation under the trade name Perhexa 3M-40.

Antioxidant: 2,2-Methylenebis(4-methyl-6-tert-butylphenol), produced by Ouchi Shinko Chemical Industry Co., Ltd. under the trade name Nocrac NS-6.

Next, the starting materials shown in Table 2 below (units: parts by weight) were intimately mixed in a twin-screw extruder at a mixing temperature of 190 to 220° C. to form an intermediate layer material and cover materials. The core described above was placed within an injection-molding mold and the intermediate layer material was injection molded around the core. The cover material was then injection molded around the resulting spherical body so as to form a cover having numerous dimples on the outside surface thereof. A non-yellowing urethane resin coating was subsequently applied to the cover surface and dried, thereby giving three-piece solid golf balls in Example 1 of the invention and in Comparative Examples 1 and 2.

TABLE 2

|                                                            |                                               | Example | Comparative Example |          |
|------------------------------------------------------------|-----------------------------------------------|---------|---------------------|----------|
|                                                            |                                               | 1       | 1                   | 2        |
| Core                                                       | Diameter (mm)                                 | 35.3    | 35.3                | 35.3     |
|                                                            | Weight (g)                                    | 27.1    | 27.1                | 27.1     |
|                                                            | Deflection (mm)                               | 4.0     | 4.0                 | 4.0      |
| Intermediate layer material                                | Hytrex 4047                                   | 100     | 100                 | 100      |
| Intermediate layer                                         | Shore D hardness                              | 40      | 40                  | 40       |
|                                                            | Specific gravity                              | 1.12    | 1.12                | 1.12     |
| Spherical body<br>(core enclosed by<br>intermediate layer) | Outside diameter (mm)                         | 38.6    | 38.6                | 38.6     |
| Cover material                                             | Himilan 1605                                  | 50      | 50                  | 50       |
|                                                            | Himilan 1706                                  | 25      | 25                  | 25       |
|                                                            | Surlyn 9945                                   | 25      | 25                  | 25       |
|                                                            | Titanium oxide                                | 2.72    | 2.8                 | 2.8      |
|                                                            | Blue pigment                                  | 0.015   | 0.035               | 0.035    |
|                                                            | Violet pigment                                | 0.088   |                     |          |
|                                                            | Yellow pigment                                | 0.0008  |                     |          |
|                                                            | Red pigment                                   |         | 0.00052             |          |
|                                                            | Magnesium stearate                            | 0.73    | 1.85                | 1.85     |
| Cover                                                      | Shore D hardness                              | 63      | 63                  | 63       |
|                                                            | Thickness (mm)                                | 2.05    | 2.05                | 2.05     |
| Finished product                                           | Diameter (mm)                                 | 42.7    | 42.7                | 42.7     |
|                                                            | Weight (g)                                    | 45.3    | 45.3                | 45.3     |
|                                                            | Deflection (mm)                               | 3.0     | 3.0                 | 3.0      |
| Evaluation tests                                           | Appearance                                    | good    | good                | ordinary |
|                                                            | Mercury vapor lamp<br>irradiation, $\Delta E$ | 2.58    | 3.41                | 3.02     |

The materials in Table 2 are described below.

- (1) Himilan 1605 (trade name): An ionomer resin which is a sodium ion-neutralized ethylene-methacrylic acid copolymer produced by DuPont-Mitsui Polymers Co., Ltd.
- (2) Himilan 1706 (trade name): An ionomer resin which is a zinc ion-neutralized ethylene-methacrylic acid copolymer produced by DuPont-Mitsui Polymers Co., Ltd.
- (3) Surlyn 9945 (trade name): An ionomer resin which is a zinc ion-neutralized ethylene-methacrylic acid copolymer produced by E.I. du Pont de Nemours and Co.
- (4) Titanium oxide: Produced by Ishihara Sangyo Kaisha, Ltd. under the trade name Tipaque R550.
- (5) Blue pigment: Produced by Holliday Pigments, Ltd. under the trade name Ultramarine Blue (Product No: EP-62; Color index name: Blue 29).
- (6) Violet pigment: Produced by Holliday Pigments, Ltd. under the trade name Ultramarine Violet (Product No: Violet 11; Color index name: Violet 15).
- (7) Yellow pigment: Produced by Dainichi Seika Colour & Chemicals Mfg. Co., Ltd. under the trade name Daipyroxide™ (Product No: Yellow #3150; Color index name: Brown 24).
- (8) Red pigment: Produced by Ciba Specialty Chemicals under the trade name Ciba CROMOPHTAL (Product No: Pink PT; Color index name: Red 122).
- (9) Magnesium stearate: Produced by NOF Corporation

The tests in Table 2 that were carried out to evaluate the golf balls are described below.

#### Deflection (mm)

This is the amount of deformation (mm) by the spherical object (core) when subjected to an increase in load from an initial load state of 98 N (10 kgf) to a final load of 1,275 N (130 kgf).

#### <sup>30</sup> Cover Resin Hardness

The Shore D hardness measured in accordance with ASTM D-2240.

#### <sup>35</sup> Appearance Test

The appearance (color) of the ball was visually rated as good (attractive) or not.

#### Mercury Vapor Lamp Test

<sup>40</sup> This test was carried out with an H400-F mercury vapor lamp manufactured by Toshiba Corporation for color fading tests. During the test, the distance between the light source and the ball was 30 cm, and the drum speed was 1 rpm. The <sup>45</sup> surface of the ball was irradiated with the mercury vapor lamp for 24 hours. The change in color at the surface of the ball before and after irradiation was measured using a color difference meter (model MSC-IS-2DH) manufactured by <sup>50</sup> Suga Test Instruments Co., Ltd., and the color difference  $\Delta E$  for the ball before and after irradiation was determined based on the Lab color system in accordance with JIS Z 8701. A smaller color difference  $\Delta E$  indicates less change in color.

<sup>55</sup> Example 2, and Comparative Examples 3 and 4

<sup>60</sup> Aside from using the cover materials shown in Table 3 below, the three-piece golf balls in Example 2 and Comparative Examples 3 and 4 were produced in the same way as in Example 1 and Comparative Examples 1 and 2. Test results for the balls thus obtained are also shown in Table 3. The numbers associated with the materials in Table 3 indicate the amounts of the respective materials in parts by weight.

TABLE 3

|                                                            |                                       | Example | Comparative Example |          |
|------------------------------------------------------------|---------------------------------------|---------|---------------------|----------|
|                                                            |                                       | 2       | 3                   | 4        |
| Core                                                       | Diameter (mm)                         | 35.3    | 35.3                | 35.3     |
|                                                            | Weight (g)                            | 27.1    | 27.1                | 27.1     |
|                                                            | Deflection (mm)                       | 4.0     | 4.0                 | 4.0      |
| Intermediate layer material                                | Hydrel 4047                           | 100     | 100                 | 100      |
| Intermediate layer                                         | Shore D hardness                      | 40      | 40                  | 40       |
|                                                            | Specific gravity                      | 1.12    | 1.12                | 1.12     |
| Spherical body<br>(core enclosed by<br>intermediate layer) | Outside diameter (mm)                 | 38.6    | 38.6                | 38.6     |
| Cover material                                             | Surlyn 8940                           | 50      | 50                  | 50       |
|                                                            | Surlyn 9910                           | 50      | 50                  | 50       |
|                                                            | Polyethylene wax                      | 2.08    | 2.08                | 2.08     |
|                                                            | Titanium oxide                        | 4.86    | 4.86                | 4.86     |
|                                                            | Blue pigment                          | 0.03    | 0.03                | 0.03     |
|                                                            | Violet pigment                        | 0.006   |                     |          |
|                                                            | Red pigment                           |         | 0.0004              |          |
|                                                            | Magnesium stearate                    | 0.32    | 0.32                | 0.32     |
| Cover                                                      | Shore D hardness                      | 63      | 63                  | 63       |
|                                                            | Thickness (mm)                        | 2.05    | 2.05                | 2.05     |
| Finished product                                           | Diameter (mm)                         | 42.7    | 42.7                | 42.7     |
|                                                            | Weight (g)                            | 45.3    | 45.3                | 45.3     |
|                                                            | Deflection (mm)                       | 3.0     | 3.0                 | 3.0      |
| Evaluation tests                                           | Appearance                            | good    | good                | ordinary |
|                                                            | Mercury vapor lamp<br>irradiation, AE | 3.30    | 4.04                | 3.64     |

The materials in Table 3 are described below.

- (1) Surlyn 8940 (trade name): An ionomer resin which is a sodium ion-neutralized ethylene-methacrylic acid copolymer produced by E.I. du Pont de Nemours and Co.
- (2) Surlyn 9910 (trade name): An ionomer resin which is a zinc ion-neutralized ethylene-methacrylic acid copolymer produced by E.I. du Pont de Nemours and Co.
- (3) Polyethylene wax: Produced by Sanyo Chemical Industries, Ltd. under the trade name Sanwax 161-P.
- (4) Titanium oxide: Same as in Table 2 above.
- (5) Blue pigment: Same as in Table 2 above.
- (6) Violet pigment: Same as in Table 2 above.
- (7) Red pigment: Produced by Ciba Specialty Chemicals under the trade name Ciba CINQUASIA (Product No: Red Y RT-759-D: Color index name: Violet 19).
- (8) Magnesium stearate: Same as in Table 2 above.

The invention claimed is:

1. A golf ball, comprising a core and a cover of one or more layer that encloses the core, wherein at least one layer of the cover is composed of 100 parts by weight of a base resin, 1 to 7 parts by weight of titanium oxide, 0.002 to 0.4 part by weight of a blue pigment and 0.0006 to 0.5 part by weight of a violet pigment, wherein the weight ratio of the blue pigment to the violet pigment is from 1:99 to 99:1, and wherein the base resin of the cover is composed primarily of a thermoplastic resin and/or a thermoplastic elastomer.
2. The golf ball of claim 1, wherein the thermoplastic resin is an ionomer resin.
3. The golf ball of claim 1, wherein the cover is coated on a surface thereof with a clear urethane coating.

4. The golf ball of claim 1, wherein the weight ratio of the blue pigment to the violet pigment is from 5:95 to 95:1.

5. The golf ball of claim 1, wherein the weight ratio of the blue pigment to the violet pigment is from 10:90 to 90:10.

6. A golf ball, comprising a core and a cover of one or more layer that encloses the core, wherein at least one layer of the cover is composed of 100 parts by weight of a base resin, 1 to 7 parts by weight of titanium oxide, 0.002 to 0.4 part by weight of a blue pigment and 0.0006 to 0.5 part by weight of a violet pigment, wherein the weight ratio of the blue pigment to the violet pigment is from 1:99 to 99:1, and wherein the at least one layer of the cover additionally contains from 0.0001 to 0.01 part by weight of a yellow pigment per 100 parts by weight of the base resin.

7. The golf ball of claim 6, wherein the base resin of the cover is composed primarily of a thermoplastic resin and/or a thermoplastic elastomer.

8. The golf ball of claim 7, wherein the thermoplastic resin is an ionomer resin.

9. The golf ball of claim 6, wherein the cover is coated on a surface thereof with a clear urethane coating.

10. The golf ball of claim 6, wherein the weight ratio of the blue pigment to the violet pigment is from 5:95 to 95:1.

11. The golf ball of claim 6, wherein the weight ratio of the blue pigment to the violet pigment is from 10:90 to 90:10.

\* \* \* \* \*